

# UNITED STATES PATENT OFFICE.

ALBERT W. SMITH AND WILLIAM R. VEAZEY, OF CLEVELAND, OHIO.

## MANUFACTURE OF METALLIC SODIUM.

1,375,330.

Specification of Letters Patent. Patented Apr. 19, 1921.

No Drawing.

Application filed July 16, 1917. Serial No. 180,742.

*To all whom it may concern:*

Be it known that we, ALBERT W. SMITH and WILLIAM R. VEAZEY, citizens of the United States, and residents of Cleveland, 5 county of Cuyahoga, State of Ohio, have jointly invented a new and useful Improvement in the Manufacture of Metallic Sodium, of which the following is a specification, the principle of the invention being 10 herein explained and the best mode in which we have contemplated applying that principle, so as to distinguish it from other inventions.

The present invention relates more particularly to the electrolytic manufacture of metallic sodium, which, as is well known, is at present extensively carried on, using caustic soda ( $NaOH$ ) as the material to be electrolyzed. Despite the extensive commercial use made of this so-called Castner process, a number of difficulties attend the electrolysis of caustic soda. Thus for example only one-half of the electric current used is employed in giving sodium, the other 25 half producing hydrogen by the electrolysis of the hydroxyl resulting from the first step. The hydrogen and oxygen that are produced from an explosive mixture, with the result that the cells when in operation 30 are continually subject to more or less dangerous explosions which at least serve to scatter fine particles of caustic in the atmosphere, if no more serious damage results. Furthermore, the metallic sodium is 35 soluble in fused sodium hydroxid, except for a relatively limited temperature range, and this adds to the difficulty of the operation by making it necessary to prevent any wide fluctuation of the temperature within the 40 cell.

By reason of the aforementioned difficulties, and for the further reason that some cheaper material than caustic would of course be desirable, a number of other compounds of sodium have heretofore been tried, but none successfully so far as we are advised. Common salt ( $NaCl$ ), which would probably afford the cheapest source, unfortunately has so high a melting point that 50 the sodium volatilizes and burns as it is formed, and the same is true of all the other available compounds or salts of sodium when used alone. It has also been attempted to work with mixtures of different salts. 55 For example, caustic soda has been added to sodium carbonate ( $Na_2CO_3$ ), which latter

alone fuses at too high a temperature, in an endeavor to obtain a lower fusing mixture; the result, however, is unsatisfactory because the caustic soda electrolyzes preferentially, and no advantage is accordingly gained. 60

The object of the present invention is to provide a suitable mixture of sodium compounds or salts for use in this electrolytic 65 process, whereby metallic sodium may be produced at a much lower cost, not only by reason of the cheapening of the source-material, but also by requiring less current and otherwise simplifying and rendering less 70 dangerous the operation itself. To the accomplishment of the foregoing and related ends, the invention, then, consists of the steps hereinafter fully described and particularly pointed out in the claims. 75

The following description sets forth in detail one approved mode of carrying out the invention, such disclosed mode, however, constituting but one of the various ways in which the principle of the invention may be 80 used.

We have discovered that sodium compounds, and specifically sodium carbonate, upon being added to sodium salts other than caustic soda, in proper proportions, will 85 give a mixture capable of fusion at a low enough temperature to avoid the vaporization and burning of the metallic sodium. At the same time, by a proper selection of these other sodium compounds, the carbonate or selected compound will electrolyze 90 preferentially, which means that it is dissociated into its constituent elements at a lower voltage than the admixed compounds.

The following examples illustrate mixtures of the sort generally referred to above, which have been found satisfactory in actual practice:—

44 parts of sodium chlorid ( $NaCl$ ) were mixed with 56 parts of potassium chlorid 100 ( $KCl$ ). This gives a mixture which fuses at approximately  $640^\circ C.$ , and from such fused mass the sodium may be electrolyzed out without serious danger of ignition, although a lower temperature would be desirable. 105

As an example of a mixture having a lower point of fusion than the one just described, 34.7 parts of sodium chlorid were added to 65.3 parts of sodium carbonate. 110 The resultant mixture has a melting point of approximately  $620^\circ C.$ , and from such

mixture the sodium carbonate will preferentially electrolyze the sodium chlorid remaining practically unchanged.

As a third example a mixture of 23.2 parts of sodium chlorid, 43.5 parts of sodium carbonate, and 33.3 parts of potassium chlorid, was made, such mixture having a melting point of approximately 565° C. From this mixture, as in the case of the second one, the sodium carbonate will be electrolyzed in preference to the other compounds present, the latter remaining as a bath or diluent for the carbonate. Of course to keep the melting point of the mixture down, it is necessary to add more of the carbonate, or other salt being electrolyzed, as the electrolysis proceeds.

Any suitable electrolytic cell may be employed in connection with the foregoing, a regular Castner caustic soda cell having been found entirely satisfactory in actual practice. With the sodium carbonate mixtures described above, it has been found possible to work with a potential of four volts between the terminals of the electric machine, indicating that only a few volts are required to effect the dissociation.

Other modes of applying the principle of our invention may be employed instead of the one explained, change being made as regards the method herein disclosed, provided the step or steps stated by any one of the following claims or the equivalent of such stated steps or steps be employed.

We therefore particularly point out and distinctly claim as our invention:

1. The method of making metallic sodium, which consists in electrolyzing sodium carbonate in a fused mixture of such salt and another salt, the ingredients being proportioned so that such mixture has a lower melting point than any of its constituents.

2. The method of making metallic sodium, which consists in electrolyzing sodium carbonate in a fused mixture of such salt and a halogen salt of sodium the ingredients being proportioned so that such mixture has a lower melting point than any of its constituents.

3. The method of making metallic sodium, 50 which consists in electrolyzing sodium carbonate in a fused mixture of such salt and sodium chlorid the ingredients being proportioned so that such mixture has a lower melting point than any of its constituents. 55

4. The method of making metallic sodium, which consists in electrolyzing sodium carbonate in a fused mixture of such salt and sodium and potassium chlorids the ingredients being proportioned so that such mixture has a lower melting point than any of its constituents. 60

5. The method of making metallic sodium, which consists in electrolyzing sodium carbonate in a fused mixture of such salt and halogen salts of potassium and sodium the ingredients being proportioned so that such mixture has a lower melting point than any of its constituents. 65

6. The method of making metallic sodium, 70 which consists in electrolyzing sodium carbonate in a fused mixture of such salt and sodium and potassium chlorids in such proportion as to give such mixture a melting point of less than 600° C. 75

7. The method of making metallic sodium, which consists in electrolyzing sodium carbonate in a fused mixture of such salt and sodium and potassium chlorids, the amount of such carbonate by weight being less than 80 the sum of the two other salts and more than either one.

8. The method of making metallic sodium, which consists in electrolyzing sodium carbonate in a fused mixture of such salt and sodium and potassium chlorids in the proportion of approximately 4 to 2 to 3 parts by weight, respectively.

9. The method of making metallic sodium, which consists in electrolyzing sodium carbonate in a fused mixture of such salt and sodium and potassium chlorids in the proportion of 43.5 to 23.2 to 33.3 parts by weight, respectively.

Signed by us, this 14th day of July, 1917. 100

ALBERT W. SMITH.  
WILLIAM R. VEAZEY.